

Patented Aug. 20, 1929.

1,725,039

# UNITED STATES PATENT OFFICE.

ROGER WILLIAMS, OF WILMINGTON, DELAWARE, ASSIGNOR, BY MESNE ASSIGNMENTS, TO ELECTRO METALLURGICAL COMPANY, A CORPORATION OF WEST VIRGINIA.

## PRODUCTION OF ALLOY-SURFACE CASTINGS.

No Drawing.

Application filed February 13, 1928. Serial No. 88,139.

This invention relates to metal castings having a body of a base metal, for example iron or steel, and a chromium-alloy surface or overlay upon and forming a unitary part 5 of the body. Such castings while of low cost compared to a casting composed throughout of chromium alloy, have at their surfaces the properties characteristic of the chromium alloy and therefore, notwithstanding their 10 lower cost, are admirably adapted to serve the purposes of all-alloy castings. Such all-alloy castings although referred to for purposes of comparison are, in the case of large castings which may weigh thousands of 15 pounds, commercially impractical, since their cost is absolutely prohibitive. The present castings not only serve in the place of small all-alloy castings but also fill the place entirely unable to be filled by large castings of 20 that type.

In the production of alloy-surface castings the desire, indeed the practical necessity, is to produce a casting with a proper depth of overlay, which overlay cannot easily be 25 chipped or scaled off, nor separated from the body casting upon bending or breaking. It is also important to produce a casting the coating of which, under the conditions to be met with in use, will not diffuse or be ab- 30 sorbed into the metal of the base casting. I have devised a method of producing chromium-alloy-surface castings which satisfactorily meet the stated, and other, desirable 35 conditions. It is a major object of the in- vention to provide such a method, and to this end, and also to improve generally upon 40 methods and castings of the character indicated, the invention consists in the various matters herein described and claimed. One 45 of the features of particular merit in the accomplishment of these ends is the use during the casting operations of a uniformity-promoting or oxide-dissolving and fusion-promoting agent which ensures the production of a completely fused and homogeneous coating, as will be discussed more fully in the course of the detailed description of the invention now to follow.

The present general procedure comprises 50 coating the surfaces of the mold, corresponding to those surfaces of the casting on which the alloy coating is desired, with a layer of coating material containing chromium with or without the admixture of other metals, or 55 of suitable particular composition to produce

the particular type of casting desired, and pouring the base metal in the coated mold. The coating may be varied from  $\frac{1}{16}$  inch or less to  $\frac{1}{4}$  inch or more in thickness. The base casting metal, on flowing into the mold, flows 60 over and melts or fuses the coating material in place, the heat of the base metal causing the chromium alloy to fuse or run together, with more or less considerable admixture of base casting metal, forming a plastic or semi-fluid 65 mass which is held in place by the pressure of the molten metal in the mold, and which sets or solidifies with the base casting itself, the two forming a definite solid body. In this procedure, there is preferably used, to 70 hold the granular or coarsely pulverous chromium in position on the mold, causing it to adhere thereto, a suitable binding agent, with which the chromium is desirably mixed; and various materials exemplified by silicate 75 of soda have heretofore been suggested for use as binding agents in procedures involving the general feature of coating the mold.

It has been found in the practice of the general method indicated that it is frequently not fully satisfactory for the production of high grade coatings and castings, since castings with their coatings not properly uniform are often produced. A probable reason for this is, I believe, that the hot casting 80 metal when it enters the mold has a chemical action upon the particles of crushed coating material, by which a film of oxide is formed on these particles; and this oxide tends to prevent the rapid and complete fusion necessary for the formation of a uniform coating. 85

Now I have found that the use of certain substances in connection with the coating material results in the production of 90 satisfactory coatings. These substances are 95 metal fluorides, e. g. sodium fluoride and calcium fluoride, also borates or the like as borax or boric acid, or compounds or mixtures containing these substances, also cryolite. Such materials apparently dissolve 100 off, or prevent the formation of, the mentioned film of oxide. Whatever the explanation, they result in a satisfactory coating. In general, then, I term these substances "uniformity promoters", "oxide preventers" 105 and "oxide dissolvers". They are desirably used to the extent of .5 to 5.0 per cent by weight of the coating material: that is to say to a given weight of coating material there is added a weight of agent equal to .5 to 5.0 per 110

cent of the said given weight. Preferably the agent is mixed directly with the coating material in a finely divided state. I have found by experiment as best, and prefer of these materials, sodium fluoride. This is preferably used in powdered condition and in the proportion of 1 to 2.5 per cent by weight. It may be added to the crushed coating material previous to the introduction of the binder, e. g., previous to the mixing of the binder with the coating material. While inorganic binders, e. g. sodium silicate, may be used, I much prefer an organic binder such, as molasses, glucose, linseed oil containing 10 to 20 per cent of dissolved rosin, etc., and have found that, generally speaking, for a chromium alloy surface of the type desired, the coating material should be crushed to ground to a size such that all the particles will pass through a 15 mesh screen and substantially all be retained on a 50 mesh screen. For general purposes I prefer to use material sized to 20 to 40 mesh. For special purposes material even as fine as 100 mesh may be used; as for example the purpose indicated in U. S. Patent No. 1,545,438, Mitchell, July 7, 1925, wherein material of this fineness is used for coating over a layer of coarse material in order to ensure that during the pouring the coating shall not be washed away.

As a specific example of procedure in accordance with the invention the following will serve:

A mold for a steel or iron casting is prepared in the customary way and the surface of this mold, while in a green state (before baking or drying) is coated to the proper depth, say  $1/8''$ , with granular chromium coating material containing 2.0% of sodium fluoride and sufficient binding material, as linseed oil, molasses, etc. of the kind specified, to form a plastic mass or mortar. This is applied with the molder's trowel evenly and in a layer of uniform thickness all over the mold surface that it is desired to coat. With a mixture of proper consistency each square foot of coating  $1/8''$  thick will contain from 1 to  $1\frac{1}{2}$  lbs. of coating material. The binder causes the coating to adhere to the sand mold surface; and after drying according to usual foundry practice, and baking to a temperature of 600 to 700° F. (the usual temperature for baking molds for iron or steel), the crushed coating material mass is so hardened and adherent to the surface of the mold that it may be brushed over by the hand without displacing or dislodging it.

The mold having been thus prepared, the base metal is poured into the mold and the casting made. Desirably, though not necessarily, the casting may be done in such manner as to give a high ferro-static pressure in the mold, as by use of a high pouring gate; e. g. a gate extending to 20 to 30 inches above the top of the mold cavity, and pouring

rapidly, e. g. using with a gate 2 to 3 inches in diameter a pouring speed of 100 pounds or more per 5 seconds, indicating approximately 4 pounds per second per square inch of area. The pouring temperature of the base metal should be sufficiently high to obtain complete fusion of the coating material. For example, in the case of steel or of ferrous alloys containing chromium and carbon, chromium and nickel, either with or without silicon, manganese, tungsten or molybdenum, (the use of such base metals in connection with the present procedure being included in the present invention) the temperature should be at least 2650° F.; and when cast iron is used as the metal for the base casting, the temperature should be high and at least 2100° F. In cases where metallic chromium is used for the coating material, rather than, say, a ferro-chromium alloy, temperatures above 3000° F. are advisable.

While, as indicated above, the coating material (together with sufficient binder to form a soft paste of the consistency of ordinary mortar, and oxide-dissolver) may be applied directly to the surface of the mold with an ordinary molder's trowel and smoothed or "slicked" into place, the coating may be applied in other ways. For instance, a sheet of fabric, such as wire gauze or textile material, of fineness and closeness of mesh sufficient to hold the crushed coating material in place may be coated with a mixture of crushed chromium alloy, with or without other metals and oxide dissolving material, and binder to the proper thickness, the coated sheet dried and fitted, and fastened to the mold or core surface as by chaplet nails, wire staples, or similar devices which will insure the coated sheet remaining in proper position and undisplaced by the molten metal while the mold is being poured. If wire gauze is used as a supporting material for the crushed coating material, this should be made of a metal, say iron, which will be fused by the molten casting metal and become incorporated with the casting or coating when the mold is being poured. In case a textile material is used, it may be ordinary cheese cloth or a similar light weight material.

Or, as another method, the coating may be sprayed on the surface of the mold or core, which may be accomplished by mixing the finely divided coating material and oxide dissolving material and forcing the mixture from a suitable nozzle by compressed air, the binder, separately introduced, being mixed with the said mixture at the moment of the mixture's ejection from the nozzle. As still another method, the dry coating material and oxide dissolving material may be spread over the surface of the mold and held in place by spraying with the binding material. In either case the whole is subsequently dried before the molten casting metal is introduced

into the mold. The junctions of such sheets or any curved surfaces are coated with the trowel by hand so as to make the whole mold coating continuous and uniform in thickness. 5 Either the spraying method or the coated-sheet method are particularly suitable as a means of saving time for coating large plane surfaces, while for more intricate molds or cores, hand coating with trowel must necessarily be used.

I have found by experiment that chromium metal in various forms and combinations may be used as a coating material: either commercially pure metallic chromium 15 containing only small proportions of iron, carbon, or other impurities, or alloys varying through the series of ferro-chromium alloys to that known as "maximum 8% carbon" ferro-chromium which contains approximately 20 65% to 70% chromium and 6% to 8% carbon, the balance iron and impurities. From a practical standpoint, however, as regards cost and quality of coating produced, I prefer to use the ordinary commercial 25 ferro-chromium known as "maximum 6% carbon" which contains approximately 65% to 70% chromium, 5% to 6% carbon, the balance iron and impurities. I find that coatings made with such material according 30 to my process show practically complete oxidation resistance at temperatures up to 1800 to 1900° F.

Not only is the invention applicable to base castings of steel, and of steel alloys 35 as above indicated, but also is applicable to base castings of cast iron. As a rule, with cast iron as the base metal the coating will be only partially fused and the particles imbedded in a complex matrix of iron and steel. 40 Such coatings, in view of the very great hardness of the ferro-chromium, will have marked abrasion resistance, both for hot and cold work and when used as a coating for the inside of ingot molds for steel will prevent 45 to a considerable extent, the cutting action of the hot metal during pouring.

As of interest I may state that metallographic examination of the coatings produced on steel castings by my process show 50 that the coating or overlay is a separate and distinct layer or veneer which is firmly adherent to the surface of the casting. With the use of low carbon steel as the base metal the coating is generally of a hypo-eutectoid

character in that there is a predominance 55 of iron-chromium solid solution with a minimum of iron-chromium carbide present. With the use of high carbon steel the character of the coating will be altered, and owing to more or less absorption of carbon from 60 the steel the coating will have a hyper-eutectoid character in which there is an excess of iron-chromium carbide. As a general rule the hypo-eutectoid coatings will be found to have greater oxidation and corrosion resistance 65 than the hyper-eutectoid, while the latter owing to the greater predominance of iron-chromium carbide will have greater abrasion and wear resisting qualities. Chemical analysis of coatings made from 6% maximum 70 carbon ferro-chromium will show an average chromium content of over 35%. Photomicrographs of sections of steel castings which have had upwards of 2000 hours service at a high temperature show the coating 75 still a distinct and separate layer adherent to the base metal with no appearance that would indicate diffusion to have taken place.

I claim:

1. A coating for molds adapted to form a homogeneous surface material alloyed with a base-metal cast in the mold which comprises metal particles containing chromium, a woven organic material, and a material capable 85 of inhibiting the formation of oxides and of promoting the uniformity of the coating.

2. A coating for molds adapted to form a homogeneous surface material alloyed with 90 a base metal cast in the mold which comprises particles of ferro-chromium and a material capable of inhibiting the formation of oxides and of promoting the uniformity 95 of the coating.

3. A coating for molds adapted to form a homogeneous surface material alloyed with a base-metal cast in the mold which comprises particles of ferro-chromium and a material comprising a chromium-oxide-dissolving 100 fluoride.

4. A coating for molds adapted to form a homogeneous surface material alloyed with a base-metal cast in the mold which comprises particles of ferro-chromium and a material comprising sodium fluoride. 105

In testimony whereof I affix my signature.  
ROGER WILLIAMS.